

## UNITED STATES PATENT OFFICE.

SAMUEL PEACOCK, OF WHEELING, WEST VIRGINIA, ASSIGNOR TO WILLIS G. WALDO,  
OF WASHINGTON, DISTRICT OF COLUMBIA.

## PROCESS OF MAKING ELEMENTAL SODIUM FROM BORAX.

No Drawing.

Application filed December 8, 1921. Serial No. 520,993.

*To all whom it may concern:*

Be it known that I, SAMUEL PEACOCK, a citizen of the United States, residing at Wheeling, in the county of Ohio and State 5 of West Virginia, have invented certain new and useful Improvements in Processes of Making Elemental Sodium from Borax; and I do hereby declare the following to be a full, clear, and exact description of the invention, such as will enable others skilled in the art to which it appertains to make and use the same.

This invention relates to a process of making elemental sodium from borax, and 15 has for its object to provide a procedure which will be more efficient in practice and less costly to carry out than those heretofore proposed.

With these and other objects in view, the 20 invention consists in the novel steps and combinations of steps constituting the process, all as will be more fully hereinafter disclosed and particularly pointed out in the claims.

25 In carrying out this invention, I take sodium tetra-borate  $\text{Na}_2\text{B}_4\text{O}_7 \cdot 10\text{H}_2\text{O}$ , commonly known as borax, finely divide the same and intimately mix it with finely divided coke, or charcoal, or other suitable carbonaceous material in proportions preferably in excess of those required by theory.

The charge thus produced is placed in a retort furnace or other suitable furnacing apparatus wherein the heat treatment will 35 take place in an atmosphere which can be positively controlled and from which the air may be excluded. The charge is now raised to a preliminary temperature of about 600° C. in order to drive off the water of crystallization, and to expel substantially all the occluded gases present, and for this purpose any suitable source of heat may be employed. The temperature of the heated charge under an exclusion of air, is next 40 raised to about 1000° C., when the breaking up of the anhydrous borax and the distillation of the elemental sodium will begin in accordance with the following equation:



It is preferred to maintain the partial pressure of the evolved gases somewhat in excess of one atmosphere in the furnace chamber in order to facilitate the vaporization and separation of the metallic sodium 55

from other charge constituents as well as its escape to suitable condensers as rapidly as it is evolved.

Of course, the higher the temperature maintained in the furnace, the more rapid 60 will be the evolution of the elemental sodium, but if the temperature is raised much above 1200° C. or 1300° C. it is found that an appreciable quantity of unconverted boron oxide,  $\text{B}_2\text{O}_3$ , distills over, unless an 65 excessive pressure is maintained in the furnace. That is to say, as no large scale furnace operation is confined to a single reaction, a considerable proportion of boron oxide is liable to be formed in some parts of 70 the furnace in accordance with the following equation:



and this said boron oxide not only contaminates the sodium, but it tends to clog the 75 passages of the apparatus. Therefore, it is preferred for economic reasons not to employ a furnace temperature higher than, say 1150° C. or 1200° C. when evolving the 80 sodium content, of the borax, under normal conditions.

If only enough carbon has been employed to satisfy the last mentioned equation, after 85 the evolution of the sodium has ceased, the furnace residue consisting of boron, boron oxide, and various impurities may be cooled, and said boron recovered in any suitable manner, or said residue may be raised to say 1300° C. or 1400° C. and said oxide recovered 90 by sublimation.

This latter method is to be preferred if the recovered boron oxide is to be employed as a raw material in the production of boron nitride, in accordance with the disclosure of 95 my Patent No. 1,464,292, dated Aug. 7, 1923, and entitled "Process of producing boron nitride," for it is found that such a distillation of the oxide from its associated impurities produces said oxide in a high state 100 of purity.

It will be observed, however, that the sodium acts cyclically in reducing all the boron oxide with which it comes into intimate contact. That is, sodium and boron oxides are probably formed as intermediate products, the sodium oxide being reduced by the carbon, and the resulting sodium reacting on the boron oxide to reform sodium oxide. The process thus continues until all 110

the boron oxide that is in contact with the sodium is used up. So that if precautions are taken to maintain an intimate contact between the reacting constituents and a fairly uniform temperature throughout the charge, very little boron oxide will be left in the furnace. On the other hand, by omitting these precautions boron oxide can be readily produced in accordance with the second equation above mentioned. As soon as all the available combined oxygen has been thus used up by the sodium and converted into carbon monoxide, the elemental sodium will sublime and be rapidly recovered in the condensers.

As elemental boron does not readily alloy with sodium, and only sublimes at about 1600° C. its recovery is easily effected, and it constitutes a valuable by-product, which lessens the cost of the sodium. That is, after separating out the sodium and any boron oxide that may have been produced, the temperature of the residue is again raised to 1600° C. or higher, whereupon the elemental boron is driven off, and recovered in condensers.

It is obvious that those skilled in the art may vary the details of the process without departing from the spirit of the invention, and therefore I do not wish to be limited to the foregoing disclosure except as may be required by the claims.

What is claimed is:

1. The process of producing elemental sodium which consists in reacting on anhy-

drous sodium tetraborate with carbon in an atmosphere substantially devoid of free oxygen at a temperature sufficient to produce said sodium but below 1300° C.; and recovering the sodium thus evolved, substantially as described.

2. The process of producing elemental sodium which consists in mixing sodium tetraborate with carbon; heating the mixture to a temperature sufficient to render the said borate anhydrous; raising the temperature to a point at which elemental sodium is produced; and recovering said sodium, substantially as described.

3. The process of producing elemental sodium from an anhydrous sodium borate which consists in mixing said borate with carbon in excess; heating the mixture in an atmosphere devoid of free oxygen to a reacting temperature to drive off the sodium in its elemental form; and recovering said sodium, substantially as described.

4. The process of producing elemental sodium and elemental boron from anhydrous sodium tetraborate which consists in adding sufficient carbon to said borate to produce said sodium and boron; raising the temperature in an atmosphere devoid of free oxygen to a reacting point; separating out the free sodium thus produced; and recovering the elemental boron left in the reacting chamber, substantially as described.

In testimony whereof I affix my signature.

SAMUEL PEACOCK.